

## UNITED STATES PATENT OFFICE.

WILBUR L. WRIGHT, OF FULTON, NEW YORK.

## COATING COMPOSITION AND PAPER MATERIAL COATED THEREWITH.

No Drawing.

Application filed May 21, 1920. Serial No. 383,166.

*To all whom it may concern:*

Be it known that I, WILBUR L. WRIGHT, a citizen of the United States of America, and resident of Fulton, Oswego County, State of New York, have invented certain new and useful Improvements in and Relating to Coating Composition and Paper Material Coated Therewith, of which the following is a specification.

10 This invention relates to certain improvements in the art of rendering paper material and the like grease and moisture proof; and the objects and nature of the invention will be readily understood by those skilled 15 in the art in the light of the following explanation of what I now believe to be preferred expression and embodiment of my invention.

An object of the invention is to provide 20 paper material embodying a greaseproof barrier that will also act as a barrier against passage of moisture, and to provide a composition for forming such barrier.

With these and other objects in view my 25 invention embodies paper material impregnated or coated with a composition insoluble in grease, and that will also serve as a barrier against passage of moisture, and also a composition for grease and water proofing 30 paper material and the like.

My invention, broadly contemplates subjecting any suitable greaseproofing body or composition to the action of some suitable agent that will act to so bind together or consolidate the greaseproofing substance on or 35 in the paper material as to render such substance capable of resisting the passage of moisture as well as grease from one side of the paper material to the other.

40 I prefer to accomplish this water proofing result by the astringent action of some suitable agent such as tannin or tannic acid, although approximately the same result can be accomplished by the coagulating action 45 of a suitable coagulant, for instance, such as acetic acid. The astringent acts to bring the composition and the fibers into such close relation as to prevent passage of moisture and the coagulant acts to bind molecules and fibers together and render the barrier 50 insoluble in water, and hence both gain the same end, i. e., render the paper material impervious to moisture.

55 My invention is applicable to various paper-material grease-proofing compositions par-

ticularly those comprising an adhesive, gelatinous or body forming solution embodying one or more ingredients to maintain the flexibility of the coating or filling formed on or in paper material by the application of the 60 composition thereto.

Such compositions can comprise a solution of casein, gelatine or other suitable adhesive, and glycerine or an emulsified oil usually a vegetable oil. Where gelatine is employed the gelatine and glycerine (or soluble oil) are dissolved in water and the resulting composition is applied hot to the paper material to form a flexible coating thereon that acts as a barrier against the 70 passage of grease.

The ingredients can be employed in approximately the proportions of gelatine from two to three hundred parts more or less; glycerine or oil from ten to one hundred 75 parts more or less, and water somewhere about one thousand parts more or less.

Where casein is used instead of gelatine, the proportion will be about as above, but a suitable alkali or the like such as ammonia 80 will be added to aid in dissolving the casein. The composition embodying casein can be applied to the paper material either hot or cold.

Other ingredients can be included to perform added functions in the composition.

These compositions are usually applied in any suitable manner or by any suitable means to form coatings on the inner surfaces of paper containers, for instance, containers 90 for food products.

The compositions can also be added to the paper stock or fibrous material in the process of making paper, so that the finished paper will be impregnated with a flexible 95 body that forms a barrier against passage of grease.

Such grease barrier forming flexible bodies or coatings, however, are generally soluble in water, and it is the purpose of my invention to so change the nature thereof (whether formed by the composition hereinbefore noted or by other compounds) as to enable such bodies to act as barriers against the passage of moisture.

This result can be attained by adding a suitable proportion of tannin (tannic acid) to the composition, or other astringent suitable for the purpose. For instance, I usually add about three per cent (more or less) 110

2  
of tannic acid to the grease proofing composition before the composition is applied to the paper material.

Approximately the same result in the matter of waterproofing the grease proof barrier, is attained by subjecting the grease proofed paper containers (or the paper material) to acetic acid fumes. In other words, after the paper material or the paper containers have been coated with the grease proofing composition, such treated paper material or containers are placed in a closed chamber and subjected to the action of acetic acid fumes for a suitable length of time, say for about thirty minutes. The acetic acid solution in the chamber (out of contact with the paper material and containers) is usually subjected to heat to accelerate the generation of fumes. This acid acts on the grease proof coating as a coagulant to render the same insoluble in water.

While I have given examples of grease proofing compositions, yet I do not wish to

limit my invention to the particular compositions named as I wish to broadly claim my invention in connection with all paper and like material grease proofing compositions and coatings or bodies to which it is applicable.

What I claim is:—

30 1. A paper container for food products having an interior flexible grease proof coating coagulated to render the same moisture proof.

35 2. A paper container embodying a grease barrier formed by a casein solution rendered moisture proof by acid.

40 3. A paper material container embodying a flexible grease proof barrier coagulated by acid to render the same moisture proof.

4. A paper material container embodying a flexible grease proof barrier rendered moisture proof by a small percentage of tannic acid.

WILBUR L. WRIGHT.